

# UNITED STATES PATENT OFFICE.

ALBRECHT SCHMIDT, OF HÖCHST-ON-THE-MAIN, GERMANY, ASSIGNOR TO FARBWERKE VORM. MEISTER LUCIUS & BRÜNING, OF HÖCHST-ON-THE-MAIN, GERMANY, A CORPORATION OF GERMANY.

## NON-EXPLOSIVE PREPARATIONS AND PROCESS OF MAKING SAME.

1,136,724.

Specification of Letters Patent. Patented Apr. 20, 1915.

No Drawing.

Application filed September 22, 1914. Serial No. 863,010.

To all whom it may concern:

Be it known that I, ALBRECHT SCHMIDT, Ph. D., chemist, a citizen of the Empire of Germany, residing at Höchst-on-the-Main, Germany, have invented certain new and useful Improvements in Non-Explosive Preparations and Processes of Making Same, of which the following is a specification.

10 In U. S. patent-application Ser. No. 792,465, filed September 29, 1913 is described a process by which non-explosive preparations can be obtained and which consists in incorporating waste-liquors from sulfite-  
15 cellulose or their essential components with nitro or dinitro or polynitro compounds, for example, such as salts of dinitro- and polynitro-phenols, of which sodium-dinitro-cresolate, sodium-dinitro-phenolate, or the like, are illustrations, such compounds being in the following specification all comprised in the term "nitro-phenol compounds."

In elaborating this invention, I have 25 found that the explosiveness of the aforesaid compounds can also be prevented by adding to them inorganic salts, such, for instance, as zinc chlorid, common salt, phosphates or the like, and that this offers the 30 further advantage that, in so far as the preparations are to be used for the preservation of wood, the inflammability of the wood is lessened by such impregnation, the respective nitro compounds producing at the 35 same time a mycocide effect. Of the inorganic salts the most suitable for carrying out my present invention are those which are known to diminish the inflammability of wood, etc.

40 In other respects the method of carrying out the new process is the same as that set forth in said U. S. patent-application Ser. No. 792,465, filed September 29, 1913. Thus, for instance, a paste is produced which is 45 capable of being transported and which—even when artificially and completely dried up—is no longer explosive, by mixing sodium dinitrophenolate, or sodium dinitrophenolate containing common salt (as 50 obtainable by treating dinitrochlorobenzene with caustic soda lye) with about the same

or one and a half times the quantity or less of zinc chlorid. By allowing the pastes thus obtained to dry at a moderately high temperature, for instance *in vacuo*, solid products are obtained which, even when suddenly heated, do not explode but only glow faintly. In cases where it is not intended to suppress entirely the explosiveness of nitro-bodies but only to diminish it, considerably less of the zinc chlorid is added.

Having now described my invention, what I claim, is:

1. The process which consists in incorporating with explosive nitro-phenol compounds having mycocide properties, fireproofing inorganic salts in quantity sufficient to render the mixture non-explosive.

2. The process of manufacturing non-explosive preparations, which consists in incorporating with alkali-nitro-phenol compounds having mycocide properties in organic salts which are capable of diminishing the inflammability of combustible material.

3. As new products, the preparations obtainable by incorporating with explosive nitro-phenol compounds having mycocide properties, fireproofing inorganic salts in quantity sufficient to render the mixture non-explosive.

4. As new products having mycocide properties, the preparations obtainable by incorporating inorganic salts with sodium-dinitro-phenolate, said preparations showing on the one hand the reactions of the sodium-dinitro-phenolate and on the other hand those of the said inorganic salts.

5. As new products having mycocide properties, the preparations obtainable by incorporating zinc chlorid with sodium-dinitro-phenolate, said preparations showing on the one hand the reactions of the sodium-dinitro-phenolate and on the other hand those of the zinc chlorid.

In testimony whereof I affix my signature in presence of two witnesses.

ALBRECHT SCHMIDT.

Witnesses:

JEAN GRUND,  
CARL GRUND.